

# United States Patent

[19]

Goto et al.

[11] 3,907,743

[45] Sept. 23, 1975

[54] MELT SPINNING METHOD OF  
POLYAMIDE YARN

|           |         |                     |           |
|-----------|---------|---------------------|-----------|
| 842,271   | 7/1960  | United Kingdom..... | 260/45.75 |
| 969,154   | 12/1950 | France .....        | 260/45.9  |
| 1,159,299 | 6/1958  | France .....        | 260/45.75 |

[75] Inventors: **Michio Goto; Shogo Ito; Atsuo Tanaka**, all of Mihara, Japan

[73] Assignee: **Teijin Limited**, Osaka, Japan

[22] Filed: **Sept. 7, 1971**

[21] Appl. No.: **178,430**

## [57] ABSTRACT

[52] U.S. Cl. .... **260/45.75 C; 260/45.7 R;**  
260/45.75 W; 260/45.85 S; 260/45.8;  
260/45.9 R

This invention involves the melt spinning of polyamide yarn containing 0.001 to 0.05% by weight of the polyamide of one or more compounds from the following group: magnesium acetate, magnesium chloride, magnesium bromide, magnesium nitride; and 0.05% to 5% by weight of one or more compounds from the following group: dithiocarbamate metallic salts, thioethers of fatty acids, 2-mercaptopbenzimidazol, 2-mercaptopbenzimidazol metallic salts, and 2,2'dibenzimidazol disulfide. The added compounds reduce the accumulation of carbonized material at the spinneret orifice.

[51] Int. Cl.<sup>2</sup> .... **C08G 85/00**

[58] Field of Search..... 260/45.75, 45.85, 45.8,  
260/45.9

## [56] References Cited

### UNITED STATES PATENTS

2,705,227 3/1955 Stamatoff..... 260/45.7

### FOREIGN PATENTS OR APPLICATIONS

650,173 1/1965 Belgium ..... 260/45.75

4 Claims, No Drawings

## MELT SPINNING METHOD OF POLYAMIDE YARN

## BACKGROUND OF THE INVENTION

This invention is concerned with the melt spinning method of polyamide. Especially, this invention is the method for preventing a single filament break produced by accumulation of carbonized volatile materials such as monomer and oligomer on the spinneret surface during the melt spinning of polyamide.

During the prolonged melt spinning of polyamide, volatile materials, such as monomer and oligomer adhere to the spinneret surface; after a time they are oxidized in high temperature surroundings and accumulate as carbonized material. This carbonized material accumulated on the spinneret surface produces a bending phenomena of the molten stream of polyamide during spinning. The end result produces drips or single filament breaks caused by the enlarging, bending and adherence of the melted polyamide on the spinneret.

For this reason, spinning must be regularly stopped for cleaning of the spinneret surface which reduces productivity.

Presently, there are various methods existing for elimination of these defects. For example, there are methods concerned with spinning equipment, such as sealing of the surface below the spinneret with non-reactive gas, changing spinneret capillary shapes, or applying silicone oil on the spinneret surface. But these methods were not giving the desired effect for the prevention of single filament breaks.

## SUMMARY OF THE INVENTION

This invention is the mixing of a magnesium salt and a sulfur containing organic ionic compound into the polyamide to reduce the accumulation of carbonized materials on the surface of the spinneret being therefore effective in prevention of a single filament break.

In other words, this invention is the melt spinning method of polyamide characterized by the melt spinning of yarn with polyamide containing 0.001 to 0.05% by weight of the polyamide of a compound selected from one or more of the following: magnesium acetate, magnesium chloride, magnesium bromide, magnesium nitride; and 0.05 to 5% by weight of a compound selected from one type or more of the following group: dithiocarbamate metallic salts, thioethers of fatty esters, 2-mercaptopbenzimidazol, 2-mercaptopbenzimidazol metallic salts, and 2,2'-dibenzimidazol disulfide.

## DESCRIPTION OF PREFERRED EMBODIMENTS

This invention is concerned with a superior effectiveness in preventing a single filament break during the melt spinning of polyamide by using especially magnesium salt and sulfur containing ionic organic compounds as previously described. The other magnesium salts, for example, combination of magnesium oxide, magnesium sulfide, etc. with the above-described sulfur containing ionic organic compounds will not give effectiveness in preventing a single filament break.

Independently applying the magnesium salts or sulfur containing ionic organic compounds used in this invention will not give full effectiveness.

A remarkable effectiveness is obtained in prevention of single filament breaks when applying the combination of both compounds of this invention.

In this invention method, the magnesium salt addition is 0.001 to 0.05% by weight to polyamide. In case of using less than 0.001% by weight results in easy occurrence of a single filament break during the spinning. 5 The use of higher than 0.05% by weight will reduce polymerization rate when added during the polymerization, or lower the viscosity when impregnated onto chips during the spinning.

The dithiocarbamate salts used in this invention 10 method are, for example, the sodium, zinc, copper, selenium, thallium salts of dithiocarbamate, such as dimethyl dithiocarbamate, diethyl dithiocarbamate, di-n-butyl dithiocarbamate, ethyl phenol dithiocarbamate.

The 2-mercaptopbenzimidazol metallic salts are, the 15 zinc, copper and magnesium salts of 2-mercaptopbenzimidazol. And, for example, the thioethers of fatty esters are dilauryl 3,3'-thiodipropionate, distearyl 3,3'-thiodipropionate, etc. The amount of addition of these organic compounds is 0.05 to 5% by 20 weight to polyamide. Use of less than 0.05% by weight results in insufficient effectiveness in prevention of single filament breaks. Use of more than 5% by weight affects physical properties of yarn, i.e. strength is lowered, therefore, such large amounts are not favorable.

25 In this method, previously described magnesium salts and organic compounds can be incorporated into the raw material of polyamide before polymerization, or added during polymerization, or mixed with polyamide chips. It follows that these additive containing polyamides will be melt spun, but the melt spinning method is not critical. Either a melter type or extruder type can be used. The extruder type is preferred because it will result in uniform yarn quality.

30 The polyamides used in this invention can be, for example, the polyamide from  $\omega$ -lactam such as poly- $\epsilon$ -caprolactam, poly- $\omega$ -nonamide, poly- $\omega$ -lauryl lactam, also the polyamides obtained from diamines and dicarboxylic acids and their copolymers or blends of various polymers of polyhexamethyleneadipamide, polyhex-35 amethylene sebacamide, polyhexamethylene isophthalamide, when these polymers can contain a luster agent, heat stabilizer, ultra violet light stabilizer, anti-static electricity agent, terminator, and optical brightener.

40 45 Based on this invention that the bending phenomena of melted polyamide on the spinneret surface is greatly reduced, furthermore remarkable extension of time for a single filament break occurs which results in a remarkable extension of time for spinneret surface cleaning cycle.

## EXAMPLES

The actual examples are as follows. In the inherent viscosity given in the examples were calculated from 55 the viscosity measurement in meta-cresol at 30°C., and the parts given in examples are all on the weight basis.

ACTUAL EXAMPLES 1-5, COMPARISON  
EXAMPLE 1-6

60 65 After polymerizing 100 parts of the  $\epsilon$ -caprolactam, and 1 part water for four (4) hours in the autoclave at 265°C., various magnesium salts and sulfur containing organic ionic compound were added, then nitrogen blanket pressure was gradually reduced.

Chips of poly- $\epsilon$ -caprolactam (inherent viscosity 1.42) using 40 grams per denier ratio extruder chips were spun with the following conditions: 280°C. spin-

ning temperature, 600 m/minute spinning speeds, 28°C. cooling air temperature and using a spinneret having 0.6 l/d ratio capillaries. The measurement of occurrence time for the bending or a single filament break was made on the first occurrence time with using 5 a previously silicone oil sprayed spinneret during spinning. The average values of measurements are shown in Table I. For comparison, poly-e-caproamide is obtained (inherent viscosity, 1.45) without using above described magnesium salts or sulfur containing organic 10 ionic compounds. The first occurrence time of the bending or a single filament break was measured. The average values of measurement are shown in Table I.

dithiocarbamate metallic salts, thiodialkanoic acid esters, 2-mercaptopbenzimidazol, 2-mercaptopbenzimidazol metal salts, and 2,2'-dibenzimidazol disulfide.

2. The method of claim 1 wherein the polyamide is polycaprolactam.

3. A method to reduce build-up of carbonized material on the surface of a spinneret during spinning of synthetic linear polyamides having recurring amide groups consisting of

TABLE I

| Actual Example     | Magnesium Salt     | (Part) | Ion Contained Organic Compound | (Part) | Occurrence Time of Bending (Hour) | Occurrence Time of Single Filament Break (Hour) |
|--------------------|--------------------|--------|--------------------------------|--------|-----------------------------------|-------------------------------------------------|
| 1                  | Magnesium Acetate  | 0.05   | Zinc diethyl dithiocarbamate   | 0.5    | 32                                | 55                                              |
| 2                  | Magnesium Nitride  | 0.03   | 2-mercaptopbenzimidazol        | 0.3    | 33                                | 58                                              |
| 3                  | Magnesium Chloride | 0.05   | Dilauryl-3,3'-thiodipropionate | 0.5    | 37                                | 63                                              |
| 4                  | Magnesium Bromide  | 0.01   | copper 2-mercaptopbenzimidazol | 0.4    | 29                                | 56                                              |
| 5                  | Magnesium Bromide  | 0.01   | 2,2'-dibenzimidazol disulfide  | 0.2    | 28                                | 55                                              |
| <hr/>              |                    |        |                                |        |                                   |                                                 |
| Comparison Example | None               | —      | None                           | —      | 7                                 | 13                                              |
| 1                  | Magnesium Nitride  | 0.03   | None                           | —      | 14                                | 23                                              |
| 3                  | Magnesium Chloride | 0.05   | None                           | —      | 15                                | 28                                              |
| 4                  | None               | —      | 2-mercaptopbenzimidazol        | 0.3    | 16                                | 30                                              |
| 5                  | None               | —      | Dilauryl 3,3'-thiodipropionate | 0.5    | 15                                | 29                                              |
| 6                  | Magnesium Oxide    | 0.05   | Zinc diethyl dithiocarbamate   | 0.5    | 15                                | 27                                              |

From Table I, it is shown the remarkable extension of a single filament break occurrence time. Again it is shown that use of other magnesium salt as used in this invention, such as magnesium oxide with sulfur containing 40 ionic organic compound will not give the superior effectiveness as the result obtained from this invention.

We claim:

1. A method to reduce build-up of carbonized material on the surface of a spinneret during spinning of synthetic linear polyamides having recurring amide groups consisting of

spinning a polyamide composition comprising a polyamide containing from about 0.001 to about 0.05% by weight of the polyamide of a compound selected 50 from the group consisting of magnesium acetate, magnesium chloride, magnesium bromide, and magnesium nitride, and

from about 0.05 to about 5% by weight of the polyamide of a compound selected from the group consisting of

spinning a polyamide composition comprising a polyamide containing from about 0.001 to about 0.05% by weight of the polyamide of a compound selected from the group consisting of

magnesium acetate, magnesium chloride, magnesium bromide, and magnesium nitride, and

from about 0.05 to about 5% by weight of the polyamide of a compound selected from the group consisting of

the sodium, zinc, copper, selenium and thallium salts of dithiocarbamate, dilauryl 3,3'-thiodipropionate, distearyl 3,3'-thiodipropionate, 2-mercaptopbenzimidazol, zinc, copper and magnesium salts of 2-mercaptopbenzimidazol, and 2,2'-dibenzimidazol disulfide.

4. The method of claim 3 wherein the polyamide is polycaprolactam.

\* \* \* \* \*